

[54] GREASE MANUFACTURE

[75] Inventor: Francis S. Sayles, Rocky Hill, N.J.

[73] Assignee: Mobil Oil Corporation, New York, N.Y.

[22] Filed: July 1, 1974

[21] Appl. No.: 484,909

[52] U.S. Cl..... 252/36; 252/40.5; 252/51.5 R;  
252/51.5 A; 252/56 R

[51] Int. Cl..... C10m 5/16; C10m 5/12

[58] Field of Search..... 252/36, 51.5 R, 51.5 A,  
252/56 R, 40.5

[56] References Cited

UNITED STATES PATENTS

3,705,853 12/1972 Fran et al. .... 252/36

Primary Examiner—Delbert E. Gantz

Assistant Examiner—I. Vaughn

Attorney, Agent, or Firm—Charles A. Huggett; Oswald G. Hayes

[57] ABSTRACT

In a process for manufacturing a calcium complex grease in which there is incorporated an ethylene-vinyl esterorganic acid terpolymer as an improving agent, a method is provided for improving grease formulation, obtaining improved yield and making use of previously unsuitable oils by introducing the terpolymer to the charge of the lubricating vehicle and thickening agent components prior to saponification.

15 Claims, No Drawings

## GREASE MANUFACTURE

## BACKGROUND OF THE INVENTION

## 1. Field of the Invention

This invention relates to grease manufacture and, in one of its aspects, relates more particularly to a process for manufacturing a calcium complex grease in which there is incorporated in the formulation an ethylene-vinyl ester-organic acid terpolymer for improving water wash-out resistance and resistance to softening at relatively high temperature environments.

## 2. Description of the Prior Art

In commonly assigned U.S. Pat. No. 3,705,853, issued Dec. 12, 1972, there are provided grease compositions having improved resistance to water wash-out and resistance to softening at high temperature conditions, comprising calcium complex greases containing ethylene-vinyl ester - organic acid terpolymers as improving agents. More specifically, the terpolymers of these formulations have a melt index of 0.5 to 200 and contain: (1) at least 65 percent, by weight, of ethylene, (2) at least 5 percent, by weight, of a second ethylenically unsaturated monomer which is an ester of the group consisting of the vinyl esters of the lower (1-6 carbon) saturated aliphatic carboxylic acids, the alkyl acrylates, the alkyl methacrylates, the dialkyl maleates and the dialkyl fumarates of the lower (1-6 carbon) aliphatic alcohols; and (3) 0.01 to 3 percent, by weight, of a third ethylenically unsaturated monomer of the group consisting of acrylic, methacrylic, itaconic, maleic and fumaric acids; the anhydrides of itaconic, maleic and fumaric acids; the alkyl hydrogen maleates and the alkyl hydrogen fumarates; the monoacrylates and monomethylacrylates of glycols; 2-hydroxy-3-amino-propyl allyl ether, allyl glycerol ether, divinyl glycol, 2-dimethylaminoethyl acrylate, 2-dimethylaminoethyl methacrylate and N-vinyl pyrrolidone. The preparation of the above-described terpolymer improving agents is more fully disclosed in U.S. Pat. No. 3,215,657, issued Nov. 2, 1965.

The thickening agents employed in the greases of the present invention comprise calcium complex soaps, including calcium acetate complex soaps and calcium-lead acetate complex soaps.

Oils used in the greases of this invention can be mineral or synthetic oils of lubricating viscosity. Suitable mineral oils have a viscosity (SUS) of at least 40 seconds at 100°F, and particularly those within the range of about 60 seconds to about 6,000 seconds at 100°F.

Synthetic vehicles can be used, instead of mineral oils, or in combination therewith. Typical synthetic vehicles are: polypropylene, polypropylene glycol, trimethylol propane esters, neopentyl and pentaerythritol esters, di(2-ethyl hexyl) sebacate, di-(2-ethyl hexyl) adipate, dibutyl phthalate, polyethylene glycol di(2-ethyl hexoate), fluorocarbons, perfluoroalkyl-polyethers, silicate esters, silanes, esters of phosphorus-containing acids, liquid ureas, ferrocene derivatives, hydrogenated mineral oils, chain type polyphenyls, siloxanes, and silicones (polysiloxanes) fluorosilicones, alkyl-substituted diphenyl ethers typified by a butyl-substituted bis-(p-phenoxy phenyl) ether, and phenoxy phenyl ethers.

Other hydrocarbon oils include synthesized hydrocarbon polymers having improved viscosity indices, which polymers are prepared by polymerizing an olefin, or mixture of olefins, having from 5 to 18 carbon

atoms per molecule in the presence of an aliphatic halide and a Ziegler-type catalyst.

With reference to the terpolymer improving agents of the present invention, preferred terpolymers contain from about 20 to about 30 percent, by weight, of the aforementioned group (2) component, i.e. the second ethylenically unsaturated monomer component; and from about 0.1 to about 1 percent, by weight, of the aforementioned group (3) component, i.e. the third ethylenically unsaturated monomer component. Representative preferred terpolymers comprise, in addition to ethylene, from about 20 to about 30 percent, by weight, vinyl acetate and from about 0.1 to about 1 percent, by weight, acrylic acid; from about 20 to about 30 percent, by weight, vinyl acetate and from about 0.1 to about 1 percent, by weight, methacrylic acid; from about 20 to about 30 percent, by weight, ethyl acrylate and from about 0.1 to about 1 percent, by weight, acrylic acid; from about 20 to about 30 percent, by weight, ethyl acrylate and from about 0.1 to about 1 percent, by weight, methacrylic acid; from about 20 to about 30 percent, by weight, methyl methacrylate, and from about 0.1 to about 1 percent, by weight, acrylic acid; and from about 20 to about 30 percent, by weight, methyl methacrylate and from about 0.1 to about 1 percent, by weight, methacrylic acid.

Insofar as the quantity of terpolymer improving agent is concerned, the latter as previously indicated, is employed in a minor amount sufficient to incorporate in the grease formulation the desired resistance to water wash-out and resistance to softening at high temperature conditions. Particularly preferred are greases in which the terpolymer is present in an amount of at least about 0.01 percent, by weight, and for most purposes, the presence of the terpolymer in an amount from about 0.1 to about 5 percent, by weight, produces highly satisfactory improved grease compositions.

In preferred modifications, the terpolymer contains from about 20 to about 30 percent, by weight, of the group (2) monomer component and from about 0.1 to about 1 percent, by weight, of the group (3) monomer component. A particularly preferred terpolymer is one having a melt index of about 6 and containing about 71.8 percent, by weight, ethylene, about 25 percent, by weight, vinyl acetate and about 0.7 percent, by weight, methacrylic acid.

In accordance with the procedure set forth in the aforementioned U.S. Pat. No. 3,705,853, the above-described greases are prepared by conventional grease manufacturing procedures which are well known to those skilled in the art. In such conventional procedures, it has heretofore been the practice to introduce the vehicle and thickening agent components into the mixing vessel or contactor. After saponification and an ultimate grease formulation has been achieved, in accordance with usual procedure, the aforementioned terpolymer is added to the finished grease to achieve the ultimate desired product. In following such procedure, however, it has been found that complete dispersion of the terpolymer is a calcium complex soap grease (including calcium acetate complex grease and calcium lead-acetate complex grease) is not achieved and, in many instances, a satisfactory yield is not obtained.

## SUMMARY OF THE INVENTION

In accordance with the present invention, it has now been found that a more complete dispersion of the

aforementioned terpolymer, improved yields are obtained and use of hitherto unsuitable oils are able to be incorporated in calcium complex greases by introducing the terpolymer in the charge of lubricating vehicle and thickening agent components prior to saponification. Those skilled in the art have long recognized the influence of oils in various soap-base systems in that calcium acetate complex and calcium lead acetate complex grease bases are affected, for example, by substituting a paraffin oil for a naphthenic base oil. Naphthenic base oils notably result in a firm-bodied soap base, thereby resulting in good yield. Paraffin oils, on the other hand, in the same soap base, yield soft-bodied bases resulting in relatively poor yields.

#### DESCRIPTION OF SPECIFIC EMBODIMENTS

In order to demonstrate the improvement realized in obtaining more complete dispersion of the aforementioned terpolymers, improvement in yield, and use of hitherto unsuitable oils are able to be incorporated in calcium complex greases by introducing the terpolymer to the charge of lubricating vehicle and thickening agent components prior to saponification, comparative data were obtained, as shown in the examples of the following Tables I and II. The grease-making technique employed in the examples of Tables I and II, in general, involves charging a contactor with appropriate amounts of fatty saponifiable material, lime, litharge, water and base oil. After saponification, the soap base is discharged to a finishing kettle. In some examples the terpolymer was added at this point, in other examples it constituted a part of the original charge to the contactor. In the former cases dehydration of the soap base is concurrent with dispersion of the terpolymer therein. Cooling, addition of various additive packages, homogenization and final addition of oil, complete the manufacture. The terpolymer employed in the examples of Tables I and II had a melt index of about 6 and contained about 71.8 percent, by weight, ethylene, about 25 percent, by weight, vinyl acetate and about 0.71 percent, by weight, methacrylic acid. The base oils employed in the examples of Table I comprised either a 500 SUS solvent naphthenic neutral oil, with a V.I. of 60 or 300 SUS solvent paraffinic neutral oil having a V.I. of 90. The base oils employed in the examples of Table II comprised either a 900 SUS solvent naphthenic neutral oil having a V.I. of 65 or a 300 SUS solvent paraffinic neutral oil having a V.I. of 90.

#### INFLUENCE OF TERPOLYMER OF YIELD (% FATTY MATERIAL) AND BASE OIL ON THE MANUFACTURE OF CALCIUM-LEAD ACETATE COMPLEX AND CALCIUM ACETATE COMPLEX GREASES

TABLE II  
CALCIUM-LEAD ACETATE COMPLEX GREASES

| Ex.                             | Ter-polymer Present | Added To         | Fatty Material % | Base Oil Type | Consistency UW/W (1)* |
|---------------------------------|---------------------|------------------|------------------|---------------|-----------------------|
| CALCIUM ACETATE COMPLEX GREASES |                     |                  |                  |               |                       |
| 1                               | No                  | —                | 13.3             | Naphthenic    | 270/320               |
| 2                               | Yes                 | Finishing Kettle | 13.3             | Naphthenic    | 250/297               |
| 3                               | Yes                 | Contactor Charge | 13.3             | Naphthenic    | 210/235               |
| 4                               | No                  | —                | 13.3             | Paraffinic    | 277/313               |
| 5                               | Yes                 | Finishing Kettle | 14.0             | Paraffinic    | 268/320               |
| 6                               | Yes                 | Contactor Charge | 10.5             | Paraffinic    | 251/276               |

(1)\* UW/W = Unworked/60 Stroke Worked, ASTM D-217

20

As will be apparent from the comparative examples of Tables I and II, significantly higher amounts of fatty material or softer consistency results are encountered in the finished grease where the terpolymer is either absent, (Examples 1 and 4 in each table), or introduced into the finished grease (Examples 2 and 5 in each table,) contrasted with the presence of significantly smaller amounts of fatty material or firmer consistency results when the terpolymer is introduced in the charge to the contactor (Examples 3 and 6 in each table).

While this invention has been described with reference to preferred compositions and components therefore, it will be understood by those skilled in the art that departure from the preferred embodiments can be effectively made and are within the scope of the specification.

I claim:

1. In a process for manufacturing a calcium complex grease in which there is incorporated an ethylene-vinyl ester-organic acid terpolymer as an improving agent, the method for improving grease formation which comprises introducing said terpolymer to the charge of lubricating vehicle and thickening agent components prior to saponification.

2. A process, as defined in claim 1, wherein the vehicle of said grease comprises a paraffinic mineral lubricating oil.

3. A process, as defined in claim 1, wherein the vehicle of said grease comprises a synthetic lubricating oil.

4. A process, as defined in claim 1, wherein said terpolymer is present in said grease in an amount of at least 0.01%, by weight.

5. A process, as defined in claim 1, wherein said terpolymer is present in said grease in an amount from about 0.1 to about 5 percent, by weight.

6. A process, as defined in claim 1, wherein said grease composition comprises a lubricating vehicle, a grease-forming quantity of a thickening agent and a minor effective amount of an improving agent comprising a terpolymer having a melt index of 0.5 to 200 and containing: (1) at least 65 percent, by weight, of ethylene, (2) at least 5 percent, by weight, of a second ethylenically unsaturated monomer which is an ester of the group consisting of: the vinyl esters of saturated aliphatic carboxylic acids having 1-6 carbons; the alkyl acrylates, the alkyl methacrylates, the dialkyl maleates

#### INFLUENCE OF TERPOLYMER OF YIELD (% FATTY MATERIAL) AND BASE OIL ON THE MANUFACTURE OF CALCIUM-LEAD ACETATE COMPLEX AND CALCIUM ACETATE COMPLEX GREASES

TABLE I  
CALCIUM-LEAD ACETATE COMPLEX GREASES

| Ex. | Ter-polymer Present | Added To         | Fatty Material % | Base Oil Type | Consistency UW/W (1)* |
|-----|---------------------|------------------|------------------|---------------|-----------------------|
| 1   | No                  | —                | 12.0             | Naphthenic    | 319/328               |
| 2   | Yes                 | Finishing Kettle | 12.0             | Naphthenic    | 267/298               |
| 3   | Yes                 | Contactor Charge | 10.5             | Naphthenic    | 280/301               |
| 4   | No                  | —                | 15.0             | Paraffinic    | 365/378               |
| 5   | Yes                 | Finishing Kettle | 15.0             | Paraffinic    | 347/361               |
| 6   | Yes                 | Contactor Charge | 11.0             | Paraffinic    | 277/295               |

and the dialkyl fumarates of aliphatic alcohols having 1-6 carbons; and (3) 0.01 to 3 percent, by weight of a third ethylenically unsaturated monomer of the group consisting of: acrylic, methacrylic, itaconic, maleic and fumaric acids; the anhydrides of itaconic, maleic and fumaric acids; the alkyl hydrogen maleates and the alkyl hydrogen fumarates; the monoacrylates and monomethacrylates of glycols; 2-hydroxy-3-aminopropyl allyl ether, allyl glycerol ether, divinyl glycol, 2-dimethylaminomethyl acrylate, 2-dimethylaminoethyl methacrylate and N-vinyl pyrrolidone.

7. A process, as defined in claim 6, wherein said terpolymer contains from about 20 to about 30 percent, by weight of the group (2) monomer component.

8. A process, as defined in claim 6, wherein the terpolymer contains from about 20 to about 30 percent, by weight, of the group (2) component and from about 0.1 to about 1 percent, by weight, of the group (3) monomer component.

9. A process, as defined in claim 6, wherein the terpolymer contains from about 20 to about 30 percent, by weight, of vinyl acetate and from 0.1 to about 1 percent, by weight, acrylic acid.

10. A process, as defined in claim 6, wherein the ter-

polymer contains from about 20 to about 30 percent, by weight, vinyl acetate and from about 0.1 to about 1 percent, by weight, methacrylic acid.

11. A process, as defined in claim 6, wherein the terpolymer contains from about 20 to about 30 percent, by weight, ethylacrylate and from about 0.1 to about 1 percent, by weight, acrylic acid.

12. A process, as defined in claim 6, wherein the terpolymer contains from about 20 to about 30 percent, by weight, ethylacrylate and from about 0.1 to about 1 percent, by weight, methacrylic acid.

13. A process, as defined in claim 1, wherein the terpolymer contains from about 20 to about 30 percent, by weight, methylmethacrylate and from about 0.1 to about 1 percent, by weight, acrylic acid.

14. A process, as defined in claim 6, wherein the terpolymer contains from about 20 to about 30 percent, by weight, methylmethacrylate and from about 0.1 to about 1 percent, by weight, methacrylic acid.

15. A process, as defined in claim 6, wherein the terpolymer has a melt index of about 6 and contains about 7.18 percent, by weight, ethylene, about 25.0 percent, by weight, vinyl acetate and about 0.7 percent, by weight, methacrylic acid.

\* \* \* \* \*

30

35

40

45

50

55

60

65

UNITED STATES PATENT AND TRADEMARK OFFICE  
CERTIFICATE OF CORRECTION

PATENT NO. : 3,904,534

DATED : September 9, 1975

INVENTOR(S) : FRANCIS S. SAYLES

It is certified that error appears in the above-identified patent and that said Letters Patent are hereby corrected as shown below:

Column 6, line 22, "7.18" should read --71.8--

Signed and Sealed this

*ninth Day of December 1975*

[SEAL]

*Attest:*

**RUTH C. MASON**  
*Attesting Officer*

**C. MARSHALL DANN**  
*Commissioner of Patents and Trademarks*